

3,758,351  
PREFERENTIAL ETCHING METHOD FOR  
FERROUS BASE METALS

Walter J. Striedieck, Port Matilda, and George Daniel Woodring, Bellefonte, Pa., assignors to Chemcut Corporation, State College, Pa.

No Drawing. Continuation-in-part of abandoned application Ser. No. 749,591, Aug. 2, 1968. This application July 15, 1971, Ser. No. 163,036

Int. Cl. C23b 3/02

U.S. Cl. 156—18

7 Claims

## ABSTRACT OF THE DISCLOSURE

Liquid compositions for etching metals and alloys and methods of etching employing these compositions are disclosed in which selected metal stock or metal objects, preferably of a ferrous base, are preferentially etched to remove portions of metal from the workpiece in the production of final etched articles. The composition contains as major ingredients a (1) pH regulator component comprising an acidic precursor and (2) an undercut protector component comprising cupric ions and/or oxygen-bearing salts of phosphorous or arsenic in particular combinations and proportions with the pH regulator. A preferred embodiment of the invention utilizes a particular combination of these components which interact compatibly to produce a synergistic effect in that a vastly superior result is obtained as compared to that which would be expected.

This is a continuation-in-part of application Ser. No. 749,591, filed Aug. 2, 1968, now abandoned.

## BACKGROUND OF THE INVENTION

For many years, etching of metal surfaces such as, for example, in the making of metal printing surfaces, has been done by coating a plate of an acid soluble metal, such as zinc and copper or alloys thereof, with a light sensitive coating. This coating was then subjected to electromagnetic radiation, such as a strong light through an image-bearing film transparency in contact with the coating or by focusing the image of the transparency thereon. The portions of the coating exposed to the light would harden and become etch resistant, while unexposed portions of the coating could subsequently be removed to reveal bare metal for etching, leaving said acid etch resistant coating as an image pattern on the plate. This image is sometimes further hardened by heating to make it more durable. The plate so prepared was then contacted with an etching solution, which attacks the bare metal portions of the metal plate not protected by the harden coating. As etching progresses, the etchant not only attacks the unprotected metal but also the side walls which begin to form about the periphery of the image areas. Accordingly, etching action also proceeds laterally and "undercuts" the coated image areas, thus producing a final article which, among other defects, no longer conforms with the original image, and is, therefore, unsuitable as a printing surface.

In the past, such undercutting was controlled by periodically interrupting the etching action and mechanically banking a deposit of a hardenable resinous powder on the formed side wall of the image, then heating to convert the powder into an etchant resistant barrier. This method of controlling undercutting, called powdering, was extremely time consuming and expensive and, therefore, in recent years has been replaced by a so called powderless process, wherein an organic film is formed on the side walls automatically during the etching operation.

The old powder process and the more recent powderless process of etching are described in detail in, for

example, U.S. Letters Patents 2,640,767, 2,828,194, and 3,152,083.

While the powderless process has been very successful and widely used, particularly in the preparation of metal relief printing plates, even to the extent of obsoleting the old powder method, it suffers the serious limitation of only being applicable to non-ferrous base metals such as zinc, copper and magnesium, and their alloys. Therefore, notwithstanding that iron and steels comprise by far the lowest cost most extensively used base metal throughout the world, ferrous base metals have not been available for the many applications which a ferrous base metal powderless etching process could make available such as listed herein before.

## DESCRIPTION OF THE INVENTION

This invention relates to new and improved powderless etching baths and to improved methods of powderless etching and particularly to novel etching baths and etching methods for use in the selective or preferential etching of a variety of things such as, for example, massive pieces or flat or curved metallic foils, sheets and plates, in the making of articles such as computer print drums, type bars, molding dies and printing plates. The invention also relates to and is useful in the field of chemical machining of metals for making such articles as templates and other blanked, contoured or perforated objects.

Accordingly, the present invention, in providing a powderless type method for etching ferrous metals represents an extremely significant and pioneering contribution to the art, in that now the basic metal of industry can be chemically processed or etched powderlessly to produce not only printing plates but numerous other articles which were heretofore only available for production by stamping or punching or mechanical machining. Moreover, the present invention has the inherent advantage of producing a totally unstressed and burr-free part or article of a ferrous base metal. It also has the added advantage of being able to powderlessly etch magnesium base metals as well as ferrous base metals.

Since the present invention has significant utility in the preparation of relief letterpress printing plates, this application has been used as a convenient means or vehicle to describe the invention and show its utility. It should be understood, however, that this invention is by no means limited to photoengraving, and actually has its greatest utility and applicability in other fields such as e.g. chemical machining and in the making by etching of mass quantities of parts and in the production of other articles such as molding dies, templates, and computer print drums and type bars, wherein either complete penetration or perforation of the workpiece is obtained by the etching action, or only a contouring or shaping effect. This invention does not relate to methods or compositions of chemical conversion coatings for the preparation or passivation of metal surfaces.

For use in describing the quality of results obtained from the present invention, a convenient measure is used herein called "etch factor" to indicate the extent of lateral attack in the direction of the image side wall. This measure is well known in the photoengraving art and as used herein is defined as the ratio of the depth of etch to the extent of undercut. The depth of etch is measured in a direction perpendicular to the etchant-resistant (simply called a "resist") coating from the surface to the bottom of the area most deeply etched adjacent to the image. The extent of undercut is the distance parallel to the coating from the original edge of the image to the top edge of the remaining metal.

An etch factor of about three is the present optimum value attainable (without any artificial side wall protec-

tion) on ferrous metals prior to the present invention. In most if not all applications, however, an etch factor of 10 or even 25 or more is required. Thus, prior to the present invention, for such applications ferrous metals have been excluded from powderless etchant use. With the advent of this invention, this limitation no longer exists since etch factors of from 4 to more than 40 can be attained together with other good and desirable characteristics of etch quality such as, e.g., cleanliness of the etched surface (little or no pimple-like defects), rapidity and uniformity of etching and a desirable shoulder angle or profile. Moreover, the present invention provides a rapid etch rate as will be shown and described herein-after.

Briefly, the present invention comprises compositions and methods for etching ferrous and magnesium metal surfaces. These compositions are aqueous solutions with a hydrogen ion concentration of 0.01 to 9 grams per liter, a lateral etch inhibitor comprised of cupric ions in a concentration of 3-140 grams per liter and an additional lateral etch inhibitor comprised of phosphate ions, in the range of 2 to 365 grams per liter, and/or arsenate ions, in the range of 1 to 365 grams per liter.

Within the foregoing range, the two preferred bath compositions (to charge a 12 gallon etcher) are:

- (1) 11.9 gallons water, 2.9 gallons 85%  $H_3PO_4$  and 14 pounds copper oxide (hereinafter sometimes referred to as a copper oxide bath) and
- (2) 9.6 gallons water, 2.4 gallons 85%  $H_3PO_4$ , 144 milliliters 42° Baumé  $HNO_3$  and 10 pounds copper nitrate (hereinafter sometimes referred to as a nitric acid bath).

The former is preferred for high carbon alloy steels, such as 52-100 (A485-3), 4720, 4730 and 1030, while the latter is preferred for low carbon steels such as SAE 1018, A181, 1018, 1006, 1008, 1010, 1015 and 1016. The latter bath (nitric acid) may not in some cases etch the high carbon or alloy steels satisfactorily.

The composition of the foregoing alloys and an indication of the source of the specifications therefor are set forth in the following table:

TABLE

|                            | C        | Si      | Mn      | Cr        | Mo      | Ni       | P <sub>max.</sub> | S <sub>max.</sub> |
|----------------------------|----------|---------|---------|-----------|---------|----------|-------------------|-------------------|
| E 52 100 (AISI) (SAE same) | .95-1.10 | .20-.35 | .25-.45 | 1.30-1.60 |         |          | .025              | .025              |
| A-485-3 (ASTM A-45)        | .95-1.10 | .20-.35 | .65-.90 | 1.1-1.5   | .20-.30 |          | .025              | .025              |
| 4720 (AISI) (SAE same)     | .17-.22  |         | .50-.70 | .35-.55   | .15-.25 | .90-1.20 |                   |                   |
| 4730 (AISI)                |          | .30     |         | .50-.70   |         |          |                   |                   |
| 1030 (AISI)                | .28-.34  |         | .60-.90 |           |         |          |                   |                   |
| 1018 (AISI) (SAE same)     | .15-.20  |         | .60-.90 |           |         |          |                   |                   |
| A-181 (ASTM)               | .35      | .35     | .90     |           |         |          | .05               |                   |
| 1006 (AISI)                | .08      |         | .25-.40 |           |         |          | .040              | .050              |
| 1008 (AISI)                | .10      |         | .25-.50 |           |         |          | .040              | .050              |
| 1010 (AISI)                | .08-.13  |         | .30-.60 |           |         |          | .040              | .050              |
| 1015 (AISI)                | .13-.18  |         | .30-.60 |           |         |          | .040              | .050              |
| 1016 (AISI)                | .13-.18  |         | .60-.90 |           |         |          | .040              | .050              |

In the method of the present invention, the baths described herein are sprayed at high pressure and close range, while at an elevated but moderate (70-140° F., preferably 70-90° F.) temperature, onto a metal plate to be etched. Ordinarily, the plate will include some masking such as patterned resist coating, to prevent etching of preselected parts of the metallic surface. In many cases, this method is used preferably in stages, i.e. the pattern is partially etched, the etchant and inhibitor are removed and the process is repeated.

The present invention may be better understood by reference to the following detailed examples and further description thereof. In all of the following examples, unless otherwise indicated, the steel etched was either 1008 or 1010 steels.

## EXAMPLE 1

A 1008 steel plate 2" x 2" was thoroughly cleaned by use of a vapor degreaser and by scouring with a cleanser grade pumice. The surface was air-blast dried. Coating with a photo-resist such as Kodak "KMER" was accomplished by slow mechanically controlled withdrawal from

70

75 An etch factor of 10 was obtained.

a reservoir. The coating was oven hardened and photo-printed by contacting the coated surface with an image bearing negative through which a strong light beam was directed. The portions of the coating exposed to the light subsequently became resistant to the developing solution which removes the unexposed coating. A final oven hardening readied the plate for etching. This plate was etched facedown in a one liter Chemcut spray etching machine equipped with Steinen number SSM-121-SQ nozzles, and operated at 120° F. with a spray pressure of 3 p.s.i. The test piece was held in position on a magnetic plate mounted within the etching apparatus. The test piece was etched for the time noted below and then washed and examined under a microscope for determination of etch factor.

The etching bath used in this example consisted of the following ingredients in the amounts indicated:

|                             |      |       |
|-----------------------------|------|-------|
| $HNO_3$ (sp. gr. 1.42)      | ml   | 3     |
| $Cu(NO_3)_2$ (19% $H_2O$ )  | gms  | 100   |
| $Na_2HPO_4$ (anhydrous cp.) | gms  | 10    |
| $H_2O$                      | ml   | 937   |
| $H^+$                       | g./l | .05   |
| $NO_3^-$                    | g./l | 55.65 |
| $PO_4^{3-}$                 | g./l | 6.7   |
| $Cu^{++}$                   | g./l | 27.2  |
| Etch depth                  | in   | .015  |

An etch factor of 15 was obtained.

## EXAMPLE 2

The procedure of Example 1 was followed using the etching bath and operating conditions set forth below:

|                               |        |       |
|-------------------------------|--------|-------|
| $HNO_3$ (sp. gr. 1.42)        | ml     | 500   |
| $Cu(NO_3)_2$ (19% $H_2O$ )    | gms    | 200   |
| $Na_2HPO_4$ (anhydrous cp.)   | gms    | 550   |
| $H_2O$                        | ml     | 250   |
| Operating machine temperature | ° F.   | 120   |
| Spray pressure                | p.s.i. | 10    |
| Etching time                  | mins.  | 20    |
| $H^+$                         | g./l   | 7.9   |
| $NO_3^-$                      | g./l   | 599.5 |
| $PO_4^{3-}$                   | g./l   | 367   |
| $Cu^{++}$                     | g./l   | 54.4  |
| Etch depth                    | in     | .025  |

An etch factor of 12 was obtained.

## EXAMPLE 3

The procedure of Example 1 was followed using the etching bath and operating conditions set forth below:

|                               |        |      |
|-------------------------------|--------|------|
| $HNO_3$ (sp. gr. 1.42)        | ml     | 140  |
| $Cu(NO_3)_2$ (19% $H_2O$ )    | gms    | 15   |
| $ZnO$ (U.S.P. powder)         | gms    | 75   |
| $H_3PO_4$ 85% (sp. gr. 1.70)  | ml     | 25   |
| $H_2O$                        | ml     | 790  |
| Operating machine temperature | ° F.   | 125  |
| Spray pressure                | p.s.i. | 13   |
| Etching time                  | mins.  | 20   |
| $H^+$                         | g./l   | 2.95 |
| $NO_3^-$                      | g./l   | 146  |
| $PO_4^{3-}$                   | g./l   | 35.1 |
| $Cu^{++}$                     | g./l   | 2.7  |
| Etch depth                    | in     | .014 |

An etch factor of 10 was obtained.

## EXAMPLE 4

The procedure of Example 1 was followed using the etching bath and operating conditions set forth below:

|                                                          |        |      |    |
|----------------------------------------------------------|--------|------|----|
| HNO <sub>3</sub> (sp. gr. 1.42)                          | ml.    | 10   | 5  |
| Cu(NO <sub>3</sub> ) <sub>2</sub> (19% H <sub>2</sub> O) | gms.   | 400  |    |
| Na <sub>2</sub> HPO <sub>4</sub> (anhydrous cp.)         | gms.   | 100  |    |
| H <sub>2</sub> O                                         | ml.    | 740  |    |
| Operating machine temperature                            | ° F.   | 120  |    |
| Spray pressure                                           | p.s.i. | 8    | 10 |
| Etching time                                             | mins.  | 10   |    |
| H <sup>+</sup>                                           | g./l.  | .16  |    |
| NO <sub>3</sub> <sup>-</sup>                             | g./l.  | 225  |    |
| PO <sub>4</sub> <sup>-3</sup>                            | g./l.  | 67   |    |
| Cu <sup>++</sup>                                         | g./l.  | 109  | 15 |
| Etch depth                                               | in.    | .025 |    |

An etch factor of 12 was obtained.

## EXAMPLE 5

The procedure of Example 1 was followed using the etching bath and operating conditions set forth below:

|                                                          |        |      |    |
|----------------------------------------------------------|--------|------|----|
| HNO <sub>3</sub> (sp. gr. 1.42)                          | ml.    | 10   | 25 |
| Cu(NO <sub>3</sub> ) <sub>2</sub> (19% H <sub>2</sub> O) | gms.   | 100  |    |
| NaHPO <sub>4</sub> (anhydrous cp.)                       | gms.   | 5    |    |
| H <sub>2</sub> O                                         | ml.    | 940  |    |
| Operating machine temperature                            | ° F.   | 120  |    |
| Spray pressure                                           | p.s.i. | 5    |    |
| Etching time                                             | mins.  | 20   | 30 |
| H <sup>+</sup>                                           | g./l.  | .16  |    |
| NO <sub>3</sub> <sup>-</sup>                             | g./l.  | 63.5 |    |
| PO <sub>4</sub> <sup>-3</sup>                            | g./l.  | 3.3  |    |
| Cu <sup>++</sup>                                         | g./l.  | 27.2 |    |
| Etch depth                                               | in.    | .022 | 35 |

An etch factor of 11 was obtained.

## EXAMPLE 6

The procedure of Example 1 was followed using the etching bath and operating conditions set forth below:

|                                                          |        |      |    |
|----------------------------------------------------------|--------|------|----|
| HNO <sub>3</sub> (sp. gr. 1.42)                          | ml.    | 3    | 45 |
| Cu(NO <sub>3</sub> ) <sub>2</sub> (19% H <sub>2</sub> O) | gms.   | 110  |    |
| Na <sub>2</sub> HAsO <sub>4</sub> (heptahydrate)         | gms.   | 25   |    |
| H <sub>2</sub> O                                         | ml.    | 920  |    |
| Operating machine temperature                            | ° F.   | 120  |    |
| Spray pressure                                           | p.s.i. | 7    |    |
| Etching time                                             | mins.  | 10   |    |
| H <sup>+</sup>                                           | g./l.  | .05  | 50 |
| NO <sub>3</sub> <sup>-</sup>                             | g./l.  | 62.1 |    |
| AsO <sub>4</sub> <sup>-3</sup>                           | g./l.  | 11.2 |    |
| Cu <sup>++</sup>                                         | g./l.  | 30.2 |    |
| Etch depth                                               | in.    | .013 |    |

An etch factor of 13 was obtained.

## EXAMPLE 7

The procedure of Example 1 was followed using the etching bath and operating conditions set forth below:

|                                                          |        |      |    |
|----------------------------------------------------------|--------|------|----|
| HNO <sub>3</sub> (sp. gr. 1.42)                          | ml.    | 500  | 60 |
| Cu(NO <sub>3</sub> ) <sub>2</sub> (19% H <sub>2</sub> O) | gms.   | 500  |    |
| NaHAsO <sub>4</sub> (heptahydrate)                       | gms.   | 600  |    |
| H <sub>2</sub> O                                         | ml.    | 100  | 65 |
| Operating machine temperature                            | ° F.   | 125  |    |
| Spray pressure                                           | p.s.i. | 2    |    |
| Etching time                                             | mins.  | 15   |    |
| H <sup>+</sup>                                           | g./l.  | 7.9  |    |
| NO <sub>3</sub> <sup>-</sup>                             | g./l.  | 761  | 70 |
| AsO <sub>4</sub> <sup>-3</sup>                           | g./l.  | 365  |    |
| Cu <sup>++</sup>                                         | g./l.  | 136  |    |
| Etch depth                                               | in.    | .015 |    |

An etch factor of 10 was obtained.

## EXAMPLE 8

The procedure of Example 1 was followed using the etching bath and operating conditions set forth below:

|                                                          |        |      |
|----------------------------------------------------------|--------|------|
| HNO <sub>3</sub> (sp. gr. 1.42)                          | ml.    | 4    |
| Cu(NO <sub>3</sub> ) <sub>2</sub> (19% H <sub>2</sub> O) | gms.   | 45   |
| Na <sub>2</sub> HAsO <sub>4</sub> (heptahydrate)         | gms.   | 15   |
| H <sub>2</sub> O                                         | ml.    | 966  |
| Operating machine temperature                            | ° F.   | 125  |
| Spray pressure                                           | p.s.i. | 10   |
| Etching time                                             | mins.  | 20   |
| H <sup>+</sup>                                           | g./l.  | .07  |
| NO <sub>3</sub> <sup>-</sup>                             | g./l.  | 28.0 |
| AsO <sub>4</sub> <sup>-3</sup>                           | g./l.  | 6.7  |
| Cu <sup>++</sup>                                         | g./l.  | 12.2 |
| Etch depth                                               | in.    | .015 |

An etch factor of 10 was obtained.

## EXAMPLE 9

The procedure of Example 1 was followed using the etching bath and operating conditions set forth below:

|                                                          |        |      |
|----------------------------------------------------------|--------|------|
| HNO <sub>3</sub> (sp. gr. 1.42)                          | ml.    | 10   |
| Cu(NO <sub>3</sub> ) <sub>2</sub> (19% H <sub>2</sub> O) | gms.   | 100  |
| Na <sub>2</sub> HAsO <sub>4</sub> (heptahydrate)         | gms.   | 5    |
| H <sub>2</sub> O                                         | ml.    | 937  |
| Operating machine temperature                            | ° F.   | 125  |
| Spray pressure                                           | p.s.i. | 10   |
| Etching time                                             | mins.  | 15   |
| H <sup>+</sup>                                           | g./l.  | .16  |
| NO <sub>3</sub> <sup>-</sup>                             | g./l.  | 63.5 |
| AsO <sub>4</sub> <sup>-3</sup>                           | g./l.  | 2.2  |
| Cu <sup>++</sup>                                         | g./l.  | 27.2 |
| Etch depth                                               | in.    | .009 |

An etch factor of 18 was obtained.

## EXAMPLE 10

The procedure of Example 1 was followed using the etching bath and operating conditions set forth below:

|                                                          |        |      |
|----------------------------------------------------------|--------|------|
| HNO <sub>3</sub> (sp. gr. 1.42)                          | ml.    | 6    |
| Cu(NO <sub>3</sub> ) <sub>2</sub> (19% H <sub>2</sub> O) | gms.   | 100  |
| Na <sub>2</sub> HAsO <sub>4</sub> (heptahydrate)         | gms.   | 5    |
| Na <sub>2</sub> HPO <sub>4</sub> (anhydrous cp.)         | gms.   | 5    |
| H <sub>2</sub> O                                         | ml.    | 937  |
| Operating machine temperature                            | ° F.   | 125  |
| Spray pressure                                           | p.s.i. | 8    |
| Etching time                                             | mins.  | 10   |
| H <sup>+</sup>                                           | g./l.  | 0.1  |
| NO <sub>3</sub> <sup>-</sup>                             | g./l.  | 59.6 |
| AsO <sub>4</sub> <sup>-3</sup>                           | g./l.  | 2.2  |
| PO <sub>4</sub> <sup>-3</sup>                            | g./l.  | 3.3  |
| Cu <sup>++</sup>                                         | g./l.  | 27.2 |
| Etch depth                                               | in.    | .018 |

An etching factor of 18 was obtained.

## EXAMPLE 11

The procedure of Example 1 was followed using the etching bath and operating conditions set forth below:

|                                                          |        |      |
|----------------------------------------------------------|--------|------|
| HNO <sub>3</sub> (sp. gr. 1.42)                          | ml.    | 500  |
| Cu(NO <sub>3</sub> ) <sub>2</sub> (19% H <sub>2</sub> O) | gms.   | 500  |
| Na <sub>2</sub> HAsO <sub>4</sub> (heptahydrate)         | gms.   | 300  |
| Na <sub>2</sub> HPO <sub>4</sub> (anhydrous cp.)         | gms.   | 300  |
| H <sub>2</sub> O                                         | ml.    | 100  |
| Operating machine temperature                            | ° F.   | 125  |
| Spray pressure                                           | p.s.i. | 2    |
| Etching time                                             | mins.  | 10   |
| H <sup>+</sup>                                           | g./l.  | 7.9  |
| NO <sub>3</sub> <sup>-</sup>                             | g./l.  | 760  |
| PO <sub>4</sub> <sup>-3</sup>                            | g./l.  | 202  |
| AsO <sub>4</sub> <sup>-3</sup>                           | g./l.  | 134  |
| Cu <sup>++</sup>                                         | g./l.  | 137  |
| Etch depth                                               | in.    | .018 |

An etch factor of 10 was obtained.

## EXAMPLE 12

The procedure of Example 1 was followed using the etching bath and operating conditions set forth below:

|                                                          |        |         |
|----------------------------------------------------------|--------|---------|
| HNO <sub>3</sub> (sp. gr. 1.42)                          | ml.    | 6       |
| Cu(NO <sub>3</sub> ) <sub>2</sub> (19% H <sub>2</sub> O) | gms.   | 50      |
| Na <sub>2</sub> HAsO <sub>4</sub> (heptahydrate)         | gms.   | 10      |
| Na <sub>2</sub> HPO <sub>4</sub> (anhydrous cp.)         | gms.   | 10      |
| H <sub>2</sub> O                                         | ml.    | 960 10  |
| Operating machine temperature                            | ° F.   | 125     |
| Spray pressure                                           | p.s.i. | 8       |
| Etching time                                             | mins.  | 10      |
| H <sup>+</sup>                                           | g./l.  | 0.1     |
| NO <sub>3</sub> <sup>-</sup>                             | g./l.  | 32.7 15 |
| AsO <sub>4</sub> <sup>-3</sup>                           | g./l.  | 4.5     |
| PO <sub>4</sub> <sup>-3</sup>                            | g./l.  | 6.7     |
| Cu <sup>++</sup>                                         | g./l.  | 13.6    |
| Etch depth                                               | in.    | .012    |

An etch factor of 12 was obtained.

## EXAMPLE 13

The procedure of Example 1 was followed using the etching bath and operating conditions set forth below:

|                                                          |        |      |
|----------------------------------------------------------|--------|------|
| HNO <sub>3</sub> (sp. gr. 1.42)                          | ml.    | 10   |
| Cu(NO <sub>3</sub> ) <sub>2</sub> (19% H <sub>2</sub> O) | gms.   | 105  |
| Na <sub>2</sub> HAsO <sub>4</sub> (heptahydrate)         | gms.   | 3    |
| Na <sub>2</sub> HPO <sub>4</sub> (anhydrous cp.)         | gms.   | 3    |
| H <sub>2</sub> O                                         | ml.    | 934  |
| Operating machine temperature                            | ° F.   | 125  |
| Spray pressure                                           | p.s.i. | 8    |
| Etching time                                             | mins.  | 10   |
| H <sup>+</sup>                                           | g./l.  | .16  |
| NO <sub>3</sub> <sup>-</sup>                             | g./l.  | 65.5 |
| AsO <sub>4</sub> <sup>-3</sup>                           | g./l.  | 1.3  |
| PO <sub>4</sub> <sup>-3</sup>                            | g./l.  | 2.0  |
| Cu <sup>++</sup>                                         | g./l.  | 28.5 |
| Etch depth                                               | in.    | .022 |

An etch factor of 11 was obtained.

## EXAMPLE 14

A high etch factor, of the order of 30 to 40, may be obtained on low carbon steels in the mode for carrying out the present invention set forth in the following example:

The procedure of Example 1 is followed using a spray etching machine operated at 125° F. and a spray pressure of 8 p.s.i. An etching time of ten minutes is employed using an etching bath consisting of the following ingredients in the amounts indicated:

|                                                          |       |       |
|----------------------------------------------------------|-------|-------|
| Cu(NO <sub>3</sub> ) <sub>2</sub> (19% H <sub>2</sub> O) | gms.  | 300   |
| Na <sub>2</sub> HAsO <sub>4</sub> (heptahydrate)         | gms.  | 125   |
| H <sub>3</sub> PO <sub>4</sub> 85% (sp. gr. 1.70)        | ml.   | 70 60 |
| H <sub>2</sub> O                                         | ml.   | 720   |
| H <sup>+</sup>                                           | g./l. | .21   |
| NO <sub>3</sub> <sup>-</sup>                             | g./l. | 161   |
| AsO <sub>4</sub> <sup>-3</sup>                           | g./l. | 56    |
| PO <sub>4</sub> <sup>-3</sup>                            | g./l. | 98    |
| Cu <sup>++</sup>                                         | g./l. | 82    |
| Etch depth                                               | in.   | .025  |

An etch factor of 35 was obtained.

## EXAMPLE 15

For the embodiment of the invention comprising hydrogen ion, cupric ion and phosphate ion, a very de-

sirable mode for carrying out the present invention is set forth in the following example:

|                                                  |        |      |
|--------------------------------------------------|--------|------|
| HNO <sub>3</sub> (sp. gr. 1.42)                  | ml.    | 3    |
| Cu(NO <sub>3</sub> ) <sub>2</sub>                | gms.   | 100  |
| Na <sub>2</sub> HPO <sub>4</sub> (anhydrous cp.) | gms.   | 10   |
| H <sub>2</sub> O                                 | ml.    | 940  |
| Operating machine temperature                    | ° F.   | 120  |
| Spray pressure                                   | p.s.i. | 3    |
| Etching time                                     | mins.  | 20   |
| H <sup>+</sup>                                   | g./l.  | .05  |
| NO <sub>3</sub> <sup>-</sup>                     | g./l.  | 56.6 |
| PO <sub>4</sub> <sup>-3</sup>                    | g./l.  | 6.7  |
| Cu <sup>++</sup>                                 | g./l.  | 27.2 |
| Etch depth                                       | in.    | .015 |

An etch factor of 15 was obtained.

## EXAMPLE 16

For the embodiment of the invention comprising hydrogen ion, cupric ion and arsenate ion, the best mode currently known to us for carrying out the present invention is set forth in the following example:

|                                                          |        |      |
|----------------------------------------------------------|--------|------|
| HNO <sub>3</sub> (sp. gr. 1.42)                          | ml.    | 10   |
| Cu(NO <sub>3</sub> ) <sub>2</sub> (19% H <sub>2</sub> O) | gms.   | 100  |
| Na <sub>2</sub> HAsO <sub>4</sub> (heptahydrate)         | gms.   | 10   |
| H <sub>2</sub> O                                         | ml.    | 1000 |
| Operating machine temperature                            | ° F.   | 125  |
| Spray pressure                                           | p.s.i. | 7    |
| Etching time                                             | mins.  | 20   |
| H <sup>+</sup>                                           | g./l.  | .16  |
| NO <sub>3</sub> <sup>-</sup>                             | g./l.  | 63.9 |
| AsO <sub>4</sub> <sup>-3</sup>                           | g./l.  | 4.5  |
| Cu <sup>++</sup>                                         | g./l.  | 27.2 |
| Etch depth                                               | in.    | .025 |

An etch factor of 12 was obtained.

## EXAMPLE 17

The procedure of Example 1 is followed using the etching bath and operating conditions set forth below:

|                                                           |        |      |
|-----------------------------------------------------------|--------|------|
| CuO                                                       | gms.   | 50   |
| H <sub>3</sub> PO <sub>4</sub> 85% (sp. gr. 1.70)         | ml.    | 125  |
| H <sub>2</sub> O in an amount sufficient to make 1 liter. |        |      |
| Operating machine temperature                             | ° F.   | 125  |
| Spray-to-work distance                                    | in.    | 4    |
| Spray pressure                                            | p.s.i. | 5    |
| Etching time                                              | mins.  | 10   |
| H <sup>+</sup>                                            | g./l.  | 3.75 |
| PO <sub>4</sub> <sup>-3</sup>                             | g./l.  | 176  |
| Cu <sup>++</sup>                                          | g./l.  | 40   |
| Etch depth                                                | in.    | .012 |

An etch factor of 36 was obtained.

## EXAMPLE 18

A highly desirable bath, insofar as etch factor is the criteria for determining desirability is set forth in the following example:

|                                                           |        |       |
|-----------------------------------------------------------|--------|-------|
| Cu(NO <sub>3</sub> ) <sub>2</sub> (19% H <sub>2</sub> O)  | gms.   | 300   |
| Na <sub>2</sub> HAsO <sub>4</sub> (heptahydrate)          | gms.   | 125   |
| H <sub>3</sub> PO <sub>4</sub> 85% (sp. gr. 1.70)         | ml.    | 75    |
| H <sub>2</sub> O in an amount sufficient to make 1 liter. |        |       |
| Metal, 1008 steel.                                        |        |       |
| Operating machine temperature                             | ° F.   | 125   |
| Spray pressure                                            | p.s.i. | 8     |
| Spray-to-work distance                                    | in.    | 6     |
| Etching time                                              | mins.  | 8     |
| H <sup>+</sup>                                            | g./l.  | 2.3   |
| NO <sub>3</sub> <sup>-</sup>                              | g./l.  | 161   |
| AsO <sub>4</sub> <sup>-3</sup>                            | g./l.  | 56    |
| PO <sub>4</sub> <sup>-3</sup>                             | g./l.  | 105   |
| Cu <sup>++</sup>                                          | g./l.  | 82    |
| Etch depth                                                | in.    | .022  |
| Undercut                                                  | in.    | .0005 |

An etch factor of 44 was obtained.

As previously indicated, the bath and the process of the present invention may be employed particularly in the field of chemical machining of metals where a vertical side wall is of greater importance than a high etch factor. The following example illustrates such use of the invention and resulted in nearly vertical side walls.

## EXAMPLE 19

|                                                           |        |      |    |
|-----------------------------------------------------------|--------|------|----|
| Cu(NO <sub>3</sub> ) <sub>2</sub> (19% H <sub>2</sub> O)  | gms    | 200  | 10 |
| Na <sub>2</sub> HPO <sub>4</sub> (anhydrous cp.)          | gms    | 140  |    |
| H <sub>3</sub> PO <sub>4</sub> 85% (sp. gr. 1.70)         | ml     | 60   |    |
| H <sub>2</sub> O in an amount sufficient to make 1 liter. |        |      |    |
| Operating machine temperature                             | ° F.   | 120  |    |
| Spray pressure                                            | p.s.i. | 12   | 15 |
| Spray-to-work distance                                    | in.    | 4    |    |
| Etching time, 10 mins. on each side.                      |        |      |    |
| H <sup>+</sup>                                            | g./l.  | 1.8  |    |
| NO <sub>3</sub> <sup>-</sup>                              | g./l.  | 107  |    |
| PO <sub>4</sub> <sup>-3</sup>                             | g./l.  | 180  |    |
| Cu <sup>++</sup>                                          | g./l.  | 54   |    |
| Etch depth                                                | in.    | .011 |    |
| Steel, 1010 CRS.                                          |        |      |    |

An etch factor of 12 was obtained.

The sample which was etched in this example was a small motor lamination. This part was etched from both sides entirely through the original metal plate—unlike the usual photoengraving examples which seek to emboss the surface. After the part was etched to the breakthrough point, it was further etched to remove the “foot” which is a result of the powderless protective process. Ideally, the product should have as nearly vertical side walls as possible. This example does present an acceptable side wall profile.

## EXAMPLE 20

An etching bath and process for the etching of magnesium photoengraving alloys (such as 3% aluminum, 1% zinc, 96% magnesium) are set forth in the following example:

|                                                            |        |      |    |
|------------------------------------------------------------|--------|------|----|
| Cu(NO <sub>3</sub> ) <sub>2</sub> (19% H <sub>2</sub> O)   | gms    | 300  | 40 |
| Na <sub>2</sub> HPO <sub>4</sub> (anhydrous cp.)           | gms    | 75   |    |
| H <sub>3</sub> PO <sub>4</sub> 85% (sp. gr. 1.70)          | ml     | 75   |    |
| H <sub>2</sub> O in an amount sufficient to make, 1 liter. |        |      |    |
| Operating machine temperature                              | ° F.   | 135  |    |
| Spray pressure                                             | p.s.i. | 1    |    |
| Spray-to-work distance                                     | in.    | 9    |    |
| Etching time                                               | mins.  | 20   | 50 |
| H <sup>+</sup>                                             | g./l.  | 2.3  |    |
| NO <sub>3</sub> <sup>-</sup>                               | g./l.  | 161  |    |
| PO <sub>4</sub> <sup>-3</sup>                              | g./l.  | 156  |    |
| Cu <sup>++</sup>                                           | g./l.  | 82   |    |
| Etch depth                                                 | in.    | .030 |    |

An etch factor of 15 was obtained.

## EXAMPLE 21

An etching bath and process for the etching of 1010 cold rolled steel are set forth in the following example:

|                                                  |        |      |    |
|--------------------------------------------------|--------|------|----|
| FeCl <sub>3</sub> (w./20 oz./gal. copper)        | ml.    | 900  | 60 |
| HNO <sub>3</sub> (sp. gr. 1.42)                  | ml.    | 180  |    |
| Na <sub>2</sub> HPO <sub>4</sub> (anhydrous cp.) | gr.    | 10   | 65 |
| Operating machine temperature                    | ° F.   | 120  |    |
| Spray pressure                                   | p.s.i. | 2    |    |
| Etching time                                     | mins.  | 10   |    |
| H <sup>+</sup>                                   | g./l.  | 3.0  | 70 |
| NO <sub>3</sub> <sup>-</sup>                     | g./l.  | 177  |    |
| PO <sub>4</sub> <sup>-3</sup>                    | g./l.  | 6.7  |    |
| Cu <sup>++</sup>                                 | g./l.  | 135  |    |
| Etch depth                                       | in.    | .006 |    |

An etch factor of 17 was obtained.

## EXAMPLE 22

The procedure of Example 1 is followed using the etching bath and operating conditions set forth below:

|   |                                                           |        |      |
|---|-----------------------------------------------------------|--------|------|
| 5 | Na <sub>2</sub> HPO <sub>4</sub> (anhydrous cp.)          | gms    | 10   |
|   | HNO <sub>3</sub> (sp. gr. 1.42)                           | ml.    | 50   |
|   | H <sub>2</sub> O in an amount sufficient to make 1 liter. |        |      |
|   | Operating machine temperature                             | ° F.   | 125  |
|   | Spray pressure                                            | p.s.i. | 8    |
|   | Spray-to-work distance                                    | in.    | 6    |
|   | Etching time                                              | mins.  | 15   |
|   | H <sup>+</sup>                                            | g./l.  | .8   |
|   | NO <sub>3</sub> <sup>-</sup>                              | g./l.  | 49   |
|   | PO <sub>4</sub> <sup>-3</sup>                             | g./l.  | 6.7  |
|   | Etch depth                                                | in.    | .006 |

An etch factor of 5 was obtained.

## EXAMPLE 23

The procedure of Example 1 is followed using the etching bath and operating conditions set forth below:

|    |                                                           |        |      |
|----|-----------------------------------------------------------|--------|------|
| 20 | Na <sub>2</sub> HAsO <sub>4</sub> (heptahydrate)          | gms    | 100  |
|    | HNO <sub>3</sub> (sp. gr. 1.42)                           | ml.    | 75   |
|    | H <sub>2</sub> O in an amount sufficient to make 1 liter. |        |      |
|    | Operating machine temperature                             | ° F.   | 125  |
|    | Spray pressure                                            | p.s.i. | 6    |
|    | Etching time                                              | mins.  | 15   |
|    | H <sup>+</sup>                                            | g./l.  | 1.18 |
|    | NO <sub>3</sub> <sup>-</sup>                              | g./l.  | 74   |
|    | AsO <sub>4</sub> <sup>-3</sup>                            | g./l.  | 67   |
|    | Etch depth                                                | in.    | .006 |

An etch factor of 9 was obtained.

It will be noted that copper is not present in either of the two foregoing baths and the reduced etch factors are thought to be a result thereof. These baths are outside the scope of the present invention and these examples are included herein for comparison only.

## EXAMPLE 24

The following example was etched in an experimental 6 liter paddle etcher such as is widely used in the photoengraving art:

|    |                                                          |        |      |
|----|----------------------------------------------------------|--------|------|
| 45 | H <sub>3</sub> PO <sub>4</sub>                           | g./l.  | 65   |
|    | Cu(NO <sub>3</sub> ) <sub>2</sub> (19% H <sub>2</sub> O) | g./l.  | 250  |
|    | Na <sub>2</sub> HAsO <sub>4</sub> (heptahydrate)         | g./l.  | 60   |
|    | Etching time                                             | mins.  | 8    |
|    | H <sup>+</sup>                                           | g./l.  | 2.0  |
| 50 | NO <sub>3</sub> <sup>-</sup>                             | g./l.  | 134  |
|    | AsO <sub>4</sub> <sup>-3</sup>                           | g./l.  | 27   |
|    | PO <sub>4</sub> <sup>-3</sup>                            | g./l.  | 92   |
|    | Cu <sup>++</sup>                                         | g./l.  | 68   |
|    | Etch depth                                               | in.    | .018 |
| 55 | Paddle speed                                             | r.p.m. | 750  |
|    | Bath temperature                                         | ° F.   | 120  |

An approximate etch factor of 15 was obtained.

## EXAMPLE 25

The following example shows the addition of Cu<sup>++</sup> to the bath in the form of CuCO<sub>3</sub>:

|    |                                |              |      |
|----|--------------------------------|--------------|------|
| 60 | CuCO <sub>3</sub>              | gms          | 100  |
|    | H <sub>3</sub> PO <sub>4</sub> | ml.          | 250  |
|    | H <sub>2</sub> O               | l. (balance) | 2    |
|    | Etching time                   | mins.        | 15   |
|    | H <sup>+</sup>                 | g./l.        | 4    |
|    | PO <sub>4</sub> <sup>-3</sup>  | g./l.        | 176  |
|    | Cu <sup>++</sup>               | g./l.        | 26   |
|    | Etch depth                     | in.          | .014 |
|    | Spray pressure                 | p.s.i.       | 4    |
|    | Temperature                    | ° F.         | 130  |

An etch factor of 7 was obtained.

**11**  
**EXAMPLE 26**

This example describes a standard etchant and its capability of etching a mild steel plate. The etch factor given is the optimum figure thought to be obtainable with this etchant.

|                                                   |        |     |
|---------------------------------------------------|--------|-----|
| FeCl <sub>3</sub> (42° Bé, circuit etching grade) | 1      | 1   |
| Etching time                                      | mins.  | 10  |
| Spray pressure                                    | p.s.i. | 15  |
| Temperature                                       | ° F.   | 130 |
| H <sup>+</sup>                                    | g./l.  | .05 |
| Fe <sup>+3</sup>                                  | g./l.  | 214 |
| Cl <sup>-</sup>                                   | g./l.  | 457 |

A maximum etch factor of 3 was obtained.

The following examples are indicative of the lower temperatures at which the etching process of the present invention may be effected. It should be noted that the preferred temperatures are in fact in this lower range.

**EXAMPLE 27**

|                                                  |              |      |
|--------------------------------------------------|--------------|------|
| Cu(NO <sub>3</sub> ) <sub>2</sub> 19%            | kg.          | 1    |
| Na <sub>2</sub> HAsO <sub>4</sub> (heptahydrate) | gms.         | 250  |
| H <sub>3</sub> PO <sub>4</sub>                   | ml.          | 300  |
| H <sub>2</sub> O                                 | l. (balance) | 5    |
| Temperature                                      | ° F.         | 100  |
| Spray pressure                                   | p.s.i.       | 4    |
| Etching time                                     | mins.        | 15   |
| H <sup>+</sup>                                   | g./l.        | 1.8  |
| NO <sup>-3</sup>                                 | g./l.        | 107  |
| AsO <sub>4</sub> <sup>-3</sup>                   | g./l.        | 22   |
| PO <sub>4</sub> <sup>-3</sup>                    | g./l.        | 84   |
| Cu <sup>++</sup>                                 | g./l.        | 54   |
| Etch depth                                       | in.          | .006 |

An etch factor of 6 was obtained.

**EXAMPLE 28**

|                                                  |              |      |
|--------------------------------------------------|--------------|------|
| Cu(NO <sub>3</sub> ) <sub>2</sub> 19%            | kg.          | 1    |
| Na <sub>2</sub> HAsO <sub>4</sub> (heptahydrate) | gms.         | 250  |
| H <sub>3</sub> PO <sub>4</sub>                   | ml.          | 300  |
| H <sub>2</sub> O                                 | l. (balance) | 5    |
| Temperature                                      | ° F.         | 110  |
| Spray pressure                                   | p.s.i.       | 40   |
| Etching time                                     | mins.        | 5    |
| H <sup>+</sup>                                   | g./l.        | 1.8  |
| AsO <sub>4</sub> <sup>-3</sup>                   | g./l.        | 22.3 |
| NO <sup>-3</sup>                                 | g./l.        | 107  |
| PO <sub>4</sub> <sup>-3</sup>                    | g./l.        | 84.2 |
| Cu <sup>++</sup>                                 | g./l.        | 54   |
| Etch depth                                       | in.          | .006 |

An etch factor of 6 was obtained.

**EXAMPLE 29**

The following example shows the results of etching with a high carbon content steel. The steel used contained 0.95% carbon.

|                                                          |              |      |
|----------------------------------------------------------|--------------|------|
| CuO                                                      | gms.         | 100  |
| Cu(NO <sub>3</sub> ) <sub>2</sub> (19% H <sub>2</sub> O) | gms.         | 100  |
| H <sub>3</sub> PO <sub>4</sub>                           | ml.          | 300  |
| H <sub>2</sub> O                                         | l. (balance) | 2    |
| Temperature                                              | ° F.         | 120  |
| Spray pressure                                           | p.s.i.       | 6    |
| Etching time                                             | mins.        | 15   |
| H <sup>+</sup>                                           | g./l.        | 1.8  |
| NO <sup>-3</sup>                                         | g./l.        | 27   |
| PO <sub>4</sub> <sup>-3</sup>                            | g./l.        | 84   |
| Cu <sup>++</sup>                                         | g./l.        | 53.6 |
| Etch depth                                               | in.          | .023 |

An etch factor of 23 was obtained.

**EXAMPLE 30**

The procedure of Example 1 was followed using the etching bath and operating conditions set forth below: This formulation is representative of an elevated etch rate

**12**

of which the present invention is capable, the etch rate being in excess of .003" per minute.

|                                                           |        |        |
|-----------------------------------------------------------|--------|--------|
| H <sub>3</sub> PO <sub>4</sub> 85% (sp. gr. 1.70)         | ml.    | 70     |
| Cu(NO <sub>3</sub> ) <sub>2</sub> (19% H <sub>2</sub> O)  | gms.   | 300    |
| Na <sub>2</sub> HAsO <sub>4</sub> (heptahydrate)          | gms.   | 100    |
| H <sub>2</sub> O in an amount sufficient to make 1 liter. |        |        |
| Temperature                                               | ° F.   | 130    |
| Spray pressure                                            | p.s.i. | 5      |
| Etch time                                                 | mins.  | 7      |
| Spray-to-work distance                                    | in.    | 4      |
| H <sup>+</sup>                                            | g./l.  | 2.1    |
| NO <sup>-3</sup>                                          | g./l.  | 161    |
| AsO <sub>4</sub> <sup>-3</sup>                            | g./l.  | 44.6   |
| PO <sub>4</sub> <sup>-3</sup>                             | g./l.  | 95.0   |
| Cu <sup>++</sup>                                          | g./l.  | 82     |
| Etch depth                                                | in.    | .024   |
| Undercut                                                  | in.    | .00075 |

An etch factor of 32 was obtained.

**EXAMPLE 31**

The foregoing examples, except Example 29, illustrate undercut inhibited etching of low carbon steels. Various special problems arise in the application of the compositions and methods of the present invention to etch, with satisfactory side wall shapes, high carbon or alloy steels. The most effective (and in some cases the only effective) etchant for these steels found to date is the copper oxide bath described above as preferred etchant 1 and also exemplified in Example 17, above.

Further, these high carbon or alloy steels must be in the "normalized" condition, as described more fully hereinafter.

Thus, by way of specific example, several samples of high carbon alloy steels, namely 52-100 (A485-3), 4720, 4730 and 1030, purchased in the "normalized" condition, were surface ground to a smoothness of 12 microinches, degreased, cleaned and covered with a patterned resist film in a conventional manner. The pattern area not covered with resist was primarily indicia, such as letters, numerals and symbols.

The etchant was prepared by adding 14 pounds copper oxide, with continuous agitation, to 2.9 gallons 85% phosphoric acid and diluting the solution with 11.9 gallons water. In an etching machine with a 12 gallon capacity, this etchant was sprayed at about 73° F. and under a pressure of 25 p.s.i., through a conical spray nozzle, commercial designation, Steinem 2688, with the work pieces at a distance of 4 inches.

An etch factor of 10:1 and an etch rate of 1/2 mil/minute were obtained with good conformance of etch shape to resist indicia characters. Among other qualitative indications of a desirable etching pattern were narrow shoulders, or relatively perpendicular side walls throughout the etching pattern.

In similar tests with other high carbon or alloy steels and with varying geometry of etch pattern, similar results have been obtained with etch factors varying from 7:1 to 10:1. Higher etch factors can also be obtained by variation of some process parameters but at the sacrifice of shoulder width which is somewhat broadened.

**EXAMPLE 32**

Ten pounds of cupric nitrate was dissolved in 9.6 gallons of water, to which was added 144 milliliters 42° Bé nitric acid and 2.4 gallons 85% phosphoric acid. This etchant was charged to an etcher having a 12 gallon capacity and used under conditions practically identical, except for spray pressure to those used in Example 31 to etch samples of several low carbon steels, namely SAE1018, A151, 1018, 1006, 1008, 1010, 1015, and 1016, all received and used in the as rolled condition and all prepared as were the samples in Example 31. With a nozzle pressure of 4 p.s.i., an etch factor of 5:1 with an etch rate of 3/4 mil/minute and relatively narrow

shoulders (straight perpendicular side walls) were obtained. Increasing the nozzle pressure to 15 p.s.i. resulted in increasing the etch rate to 1 mil/minute and decreasing the etch factor to 3:1. The shoulders or side walls remained straight, however.

This is consistent with experience in the powderless etching art generally which indicates that high pressures tend to reduce the amount of coating which is responsible for side wall protection. The result is steeper side walls as well as some sacrifice in etch factor. Correspondingly, lower pressures tend to produce broader side wall configurations with a general tendency toward slightly improved etch factors.

The foregoing preferred baths set forth in Examples 31 and 32 are calculated to have the following anionic contents:

|                   | H <sup>+</sup> | PO <sub>4</sub> <sup>-3</sup> | Cu <sup>+2</sup> |
|-------------------|----------------|-------------------------------|------------------|
| Example 31, g./l. | 8.55           | 273.6                         | 89.5             |
| Example 32, g./l. | 8.63           | 271.7                         | 26.6             |

The ranges of ionic concentration established by all of the foregoing examples therefore are as follows:

|                               |          |
|-------------------------------|----------|
| H <sup>+</sup>                | 0.5-8.63 |
| PO <sub>4</sub> <sup>-3</sup> | 3.3-357  |
| Cu <sup>+2</sup>              | 26-109   |

Generally, as indicated by the preferred baths of Examples 31 and 32, the preferred ionic concentration ranges are:

|                               |         |
|-------------------------------|---------|
| H <sup>+</sup>                | ca. 8.6 |
| PO <sub>4</sub> <sup>-3</sup> | 270-275 |
| Cu <sup>+2</sup>              | 25-90   |

As is evident from the foregoing examples, the powderless etching baths of this invention contain two major classes of components: (1) pH regulators, and (2) lateral etch minimizing agents.

A variety of pH regulators may be used to supply or remove hydrogen ions to maintain the bath preferably over a range of 0.1 to 2.0. Although the examples show only the use of nitric and phosphoric acids which are preferred, it must be understood that the pH regulators are not restricted to these materials but may also be other acids, such as hydrochloric, hydrofluoric, perchloric and sulfuric (used either singly or in combinations); acid salts, such as ferric chloride, ferric nitrate, aluminum nitrate and zinc nitrate; or buffer salts such as ammonium citrate, ammonium acetate and sodium tartrate.

The lateral etch minimizing agents which have been found effective are of two types: (1) those which produce a metallic deposit on the workpiece, such as copper; (2) those which produce a thixotropic gelatinous, non-metallic coating on the surface, such as phosphates and arsenates. The above described lateral etch minimizing agents are used in combination. The metallic coating former is copper ion in concentrations ranging from 3 to 140 grams per liter. Although the sources of copper ions shown in the examples are restricted to cupric nitrate, cupric oxide and metallic copper, it must be understood that other salts may also be successfully used such as cupric carbonate, cupric sulfate, cupric hydroxide, cupric chloride and cupric acetate.

The inorganic gelatinous coating formers are essentially phosphates and arsenates. Phosphorous compounds which have been found to be satisfactory sources of phosphate ion are phosphoric acid, the mono, di and tri-sodium orthophosphates, sodium hexametaphosphate, tetra-sodium pyrophosphate, phosphorous trioxide, phosphorous pentoxide, zinc phosphate, lithium phosphate, mono-, di- and

tri-sodium phosphates, mono-, di- and tri-ammonium phosphates and manganese phosphate. Any phosphorous compound which reverts to orthophosphate ion under operating bath make-up conditions to provide phosphate ion concentrations in the range of 2 to 365 grams per liter can be expected to perform satisfactorily.

Arsenic compounds which have been found to be acceptable sources of arsenate ion are mono-, di- and tri-sodium arsenates; mono-, di- and tri-potassium arsenates; sodium, potassium and ammonium meta-arsenites; arsenic oxide; mono-, di- and tri-ammonium arsenates, arsenous oxide; and basic copper arsenate. Any arsenate compound which reverts to orthoarsenate ion under operating bath make-up conditions to provide arsenate ion concentrations in the range of 1 to 365 grams per liter can be expected to perform satisfactorily.

Practical usage of these baths demands that operating temperatures be selected to produce the most rapid etch rates possible while permitting adequate control of the process. While it is possible to get etching action at temperatures as low as 40° F., the most practical operating temperatures range from 70° to 140° F., with 70° to 90° F. being preferred. Satisfactory etching can be attained at higher temperatures up to the boiling point, but practical upper temperature limits are governed by the corrosion resistance and temperature limitations of the equipment in which the bath is being used.

Many of the baths of the present invention, particularly those of the copper oxide variety, require agitation, and sometimes severe agitation, to keep them in sprayable form.

For proper operation of this bath, it is necessary to apply the etchant forcefully to the workpiece surface. The direction of force should be as nearly perpendicular as possible. There are several methods for impinging the etchant on the surface of the workpiece. For example: (1) Spray etching has been the method most widely employed with these baths and offers the most satisfactory control of impingement force and direction. (2) Paddle etching which, in the prior photoengraving art, has won highest acceptance and has also proved satisfactory with the baths of this invention. (3) It is possible to apply etchant forcefully to the surface of a workpiece by methods other than these two; such means may include ultrasonic agitation, for example. Whichever method is employed, the agitation of the entire mass of the bath must be sufficiently vigorous to prevent the thixotropic baths from becoming gelled. The principles of selection of nozzle configuration, spray pressures and impingement forces are no different from those utilized with conventional baths by persons skilled in the art. Similarly, side wall etching, even though substantially inhibited, will occur to different degrees depending on specific process conditions. As in conventional powderless etching, this can be compensated for by making the image slightly smaller than the actual size desired in the finished etch.

In some cases, the etching process of the present invention may slow considerably or stop altogether if continued for an extended period of time. In such cases and also in other special cases where certain etch geometry is desired, the method of the present invention may be used repeatedly or in conjunction with other etch processes, such as inhibited ferric chloride etching, conducted serially. Between steps of these multi-step procedures, the workpiece is thoroughly cleaned and all inhibitor and etchant is removed.

The mechanism responsible for the desirable results obtained by incorporating phosphate and/or arsenate ions in an etching bath containing cupric ions is not fully understood. Very shortly after the workpiece metal is exposed to the etching action, the bath also dissolves ions of the metal being etched, and a number of chemical changes and reactions are initiated involving all these ions. While the exact nature of these reactions is not

known, certain physical changes have been noted. For example, with the baths containing phosphate or arsenate there is a gradual change to a thixotropic state, so that with a particular type of agitation there is a progressive thickening of the bath as the etching proceeds. The precise role of the cupric ion in these reactions is also not known, but we have determined that the synergistic effect of the present invention is not obtained if the cupric ion is omitted. Likewise, the effect is not obtained if no phosphate or arsenate ion is included.

From the examples it will be noted that the aqueous etching baths of the present invention are characterized by the presence of at least one pH regulator selected from the group consisting of inorganic acids and acid salts which in water solution dissociate to form hydrogen ions; and at least one lateral etch minimizing agent selected from the group consisting of chemical elements, salts, acids and acid anhydrides which in acidic water solution dissociate into ions which are members of the group consisting of copper, phosphate and arsenate ions. A satisfactory concentration range for the hydrogen ion is from about 0.01 grams per liter to 8 grams per liter and a satisfactory concentration range for the cupric ion is from about 3 grams per liter to about 140 grams per liter. A satisfactory concentration range for phosphate ions is from about 2 grams per liter to about 365 grams per liter, and for arsenate ion it is from about 1 gram per liter to about 365 grams per liter.

As far as is known the upper limit of phosphate and arsenate is set only by the solubility of these ions. High copper content will lead to copper plating throughout the etch surface and substantially inhibit all etching. High copper content may be compensated for by ferric ions in solution, however. For this purpose, and sometimes to catalyze the initiation of the etching process when it is slow in starting for some other reason, iron ions or a piece of iron may be added to the etchant bath. Alternatively, a new bath may be seeded with a portion of an old bath for the same purpose.

As indicated in Example 31 above, when high carbon or alloy steels, such as 52-100 (A485-3) 4720, 4730 and 1030 are used, the steels must generally be in "normalized" condition.

Thus the steel is neither in the full hard nor full soft condition. Steels which have been hardened, such as by rolling or roll straightening, may be "normalized" by heating to a temperature about 100° F. above the critical temperature range for that steel and then cooled to below that range in still air. This produces a generally fine pearlite structure which is etchable in accordance with the present invention. Hardened steel has a martensitic structure which is not etchable, with proper side wall control and undercut inhibition, by the compositions and methods of the present invention.

No comparable problem is found in low carbon steels which may generally be etched in the as produced or annealed condition. With all steels, however, care must be taken to ensure that the surface to be etched is in proper condition. Any machining with cutting tools must be such that no cold flow or working of the metal occurs to any great depth. Cutting to a depth of about .010 inch is considered the acceptable maximum. Generally the surface is ground to remove 0.010 to 0.015 inch and to produce a finish no coarser than 12 microinches. The surface is then thoroughly cleaned prior to resist application.

While the present invention has been described by particular reference as applied to workpieces of particular ferrous alloys, including silicon steels and carbon steels and magnesium alloy plates, by means of spray and paddle etchers, it is to be understood as not being restricted to these particular alloys containing iron or magnesium, or to these particular methods of etching or chemical machining or chemical milling. Where the term "inorganic" is used in the specification and claims, it is intended

that the corresponding acetates shall be included since the active portion of the molecule gives the desired ions on dissociation in aqueous solution.

We claim:

- 5 1. A method of preferentially etching surfaces of certain carbon steels or low alloy steels containing molybdenum, chromium or nickel or mixtures thereof which comprises: providing a liquid aqueous etching composition comprising (1) at least one pH regulator selected from the group consisting of nitric, phosphoric, hydrochloric and sulfuric acids which in water solution dissociate to form hydrogen ions in a hydrogen ion concentration within the range of about 0.01 to about 9 grams per liter of bath, (2) at least one lateral etch minimizing agent selected from chemical precursors which in acidic solution forms cupric ions in a concentration of from about 3 to as much as about 140 grams per liter of bath, and (3) an additional lateral etch minimizing agent selected from the group consisting of soluble inorganic phosphates and arsenates which, in acidic solution, form at least one of the following, arsenate ions in a concentration of from about 1 to as much as about 365 grams per liter of bath and phosphate ions in a concentration of from about 2 to as much as about 365 grams per liter of bath, the total concentration of said cupric, arsenate and phosphate ions when used in combination being limited to a compatible amount to permit reasonable contact of the composition with the steel workpiece to be etched and to produce the desired quality of etch, the balance of the bath being essentially water, forcefully contacting the etching composition, at a temperature within the range of from about 70 to about 140° F., with at least a portion of the steel surface to be etched, said surface having an etch-resistant pattern thereon, continuing said contact of the etchant composition and steel surface for a period to obtain the desired degree of etching effect, whereby the areas of said surface not covered by said etch-resistant pattern are etched as a protective coating, formed from said cupric and said phosphate or arsenate ions in said composition is deposited on the sidewalls of said etch-resistant pattern.
- 10 2. The method of claim 1 wherein said composition temperature is approximately 70-90° F.
- 15 3. A method of preferentially etching low carbon steels, with inhibited undercut and side wall etching, said method comprising forcefully contacting an etching composition, said composition consisting, per gallon of solution, of
- 20
- 25
- 30
- 35
- 40

50 42° Baumé nitric acid=12 milliliters  
85% phosphoric acid=.20 gallon  
.833 pounds copper nitrate  
Balance=water

55 at a temperature in the range of 70-140° F. with at least a portion of the surface of the low carbon steel to be etched, said surface having an etch-resistant pattern thereon, continuing said contact of the etchant composition and workpiece for a period to obtain the desired degree of etching effect.

60 65 4. A method of preferentially etching high carbon steels, with inhibited undercut and side wall etching, said method comprising forcefully contacting an etching composition, said composition consisting, per gallon of solution, of

85% phosphoric acid=0.24 gallon  
1.17 pounds per cupric oxide  
Balance=water

70 at a temperature in the range of 70-140° F. with at least a portion of the surface of the high carbon steel to be etched, said surface having an etch-resistant pattern thereon, continuing said contact of the etchant composition and workpiece for a period to obtain the desired degree of etching effect.

5. A method, as recited in claim 4, wherein said additional lateral etch minimizing agent is a soluble inorganic phosphate.

6. A method, as recited in claim 5, wherein the cupric ion concentration is in the range 25-90 grams per liter.

7. A method, as recited in claim 6, wherein said phosphate ion concentration is in the range 270-275 grams per liter, and said hydrogen ion concentration is approximately 8.6 grams per liter.

**References Cited**

**UNITED STATES PATENTS**

3,193,423 7/1965 Goffredo 156—18

**FOREIGN PATENTS**

92,384 12/1961 Denmark 156—20

**OTHER REFERENCES**

5 Striecher: "Phosphatization of Metallic Surfaces," pp. 61-69 of Metal Finishing, August 1948.

Chukhlantsev et al.: pp. 706-709, Izvest Vysshii Kh Ucheb Zavedenii Khimi Khim. Tekhnol., vol. 14 (1961).

10 GEORGE F. LESMES, Primary Examiner

R. J. ROCHE, Assistant Examiner

**U.S. Cl. X.R.**

156—14; 252—79.2

UNITED STATES PATENT OFFICE  
CERTIFICATE OF CORRECTION

Patent No. 3,758,351

Dated September 11, 1973

Inventor(s) Walter J. Striedieck and George Daniel Woodring

It is certified that error appears in the above-identified patent and that said Letters Patent are hereby corrected as shown below:

35 U.S.C. 254

Column 5, Example 6, line 53, change "Cu<sup>++</sup> ---- g./l --- 30.2"  
to --Cu<sup>++</sup> ---- g./l --- 30.0--

Column 5, Example 7, line 64, change "NaHAsO<sub>4</sub> to --Na<sub>2</sub>HAsO<sub>4</sub>--

Column 6, Example 8, line 5, change "(19 /H<sub>2</sub>O)" to --(19% H<sub>2</sub>O)--

Column 6, Example 11, line 62, change "Na<sub>2</sub>NAsO<sub>4</sub>" to --Na<sub>2</sub>HAsO<sub>4</sub>--

Column 9, Example 21, line 71, change "PO<sub>4</sub>" to --PO<sub>4</sub><sup>-3</sup>--

Column 11, Example 27, line 29, change "NO<sub>3</sub>" to --NO<sub>3</sub><sup>-</sup>--

Column 13, line 15, change "anionic" to --ionic--

Column 14, line 48, change "thioxotropic" to --thixotropic--

Column 17, Claim 5, line 1, change "claim 4" to --claim 1--

Signed and sealed this 25th day of December 1973.

(SEAL)

Attest:

EDWARD M. FLETCHER, JR.  
Attesting Officer

RENE D. TEGTMEYER  
Acting Commissioner of Patents